# EUROPEAN PATENT SPECIFICATION

(11) **EP 0 054 374 B1**
(45) Date of publication and mention of the grant of the patent: **13.03.1985**
(21) Application number: 81305642.1
(22) Date of filing: 27.11.1981
(51) Int. Cl.: B21C 23/22, B21K 21/08, H01T 13/20

(54) **Spark plug electrode and its method of manufacture**
Zündkerzenelektrode und Verfahren zu ihrer Herstellung
Electrode de bougie et procédé pour sa fabrication

(30) Priority: 10.12.1980 GB 8039567
(43) Date of publication of application: 23.06.1982
(73) Proprietor: FLOFORM LIMITED, Welshpool Powys, SY21 7BJ (GB)
(72) Inventor: Howard, Kenneth, Guildsfield Welshpool (GB)
(74) Representative: Cole, Paul Gilbert

## Description

This invention relates to a method of making a spark plug centre electrode having an inner core of a metal which has good thermal conductivity relative to the metal of an outer sheath fully enclosing the inner core, the outer sheath being formed of a corrosion resistant material.

It is known to provide a spark plug electrode in which an inner core of a metal having good thermal conductivity, for example copper, is partly encased within a sheath of a metal having good corrosion resistance properties, such as for example nickel or a nickel alloy. The purpose of using a composite electrode of this type is that, while good heat conduction is required of the electrode in order to prevent undue "burning", it is also necessary to provide for a hardwearing portion of the electrode at and around the point where sparking occurs. Thus, the advantage of a composite electrode as described is that a material suitable for good heat conduction is used in conjunction with a material having suitably hardwearing properties.

For example, GB-A-754,591 discloses a method of making a spark plug electrode in which a billet of copper is placed on top of a billet of nickel, the composite billet then being extruded through a suitable die to form a spark plug electrode having at one end a core of metal having good thermal conductivity surrounded by a sleeve of the corrosion resistant metal.

In our earlier British patent application number 2037190 there is shown a method of making a composite centre electrode for a spark plug in which an outer sheath of a nickel alloy has an inner core of copper, the improvement being in the method of bonding the copper to the nickel alloy prior to extrusion.

A method of making a centre electrode for a spark plug is taught in DE-A-2238283 which involves forming a composite billet from a core billet of copper that fits into a cup-shaped billet of nickel and then extruding the composite billet to form an elongate rod-shaped extrusion whose tip portion consists solely of nickel and an intermediate portion of which consists of copper sheathed with nickel. But at the base of the electrode is exposed copper which is undesirable because it does not facilitate welding to a wire connector by electric butt welding or friction welding.

It is an object of the present invention to provide a method of making a composite centre electrode for a spark plug which electrode can be easily connected to a wire extending through the spark plug body by relatively simple welding techniques of known type, and in which the volume of copper within the electrode is carefully controlled. A further object of the invention is to provide a centre electrode for a spark plug which can be easily formed at one end to provide a shoulder for mounting in the body a spark plug.

According to one aspect of the invention there is provided a method of the kind described in DE-A-2238283 of making a centre electrode for a spark plug of the type having a core 12 of a first metal within a sheath 10 of a second metal, the first metal having a thermal conductivity higher than that of the second metal and a melting point lower than that of the second metal, the second metal being resistive to the corrosive environment in which the electrode works comprising inserting a billet 12 of the first metal within a cup-shaped billet 10 of the second metal and extruding the composite billet to form an elongate rod-shaped extrusion a tip portion of which consists solely of the second metal and an intermediate portion of which consists of said first metal enclosed in said second metal characterised in that:
(a) the two billets (10, 12) are heated together to a temperature at or above the melting point of the first metal but below the melting point of the second metal;
(b) the amount of said first metal (12) in said composite billet is such that when molten it occupies less than the whole of the depth of the cup in said billet (10) of said second metal;
(c) the two metals are cooled to a temperature below the melting point of the first metal to form a composite billet in which the first and second metals are united at their interface; and
(d) when the composite billet is extruded the base portion (24, 25) of the resulting rod-shaped extrusion consists essentially of said second metal whereby the product of said extrusion is a core of the first metal enclosed substantially entirely within a sheath of the second metal.

The heating of the first and second metals may conveniently take place in a reducing atmosphere within a radiant furnace, the cup-shaped billet of the second metal being held in a suitably shaped black body so that conduction of heat from the radiant furnace occurs through the black body in order to melt the billet of said first contained within the cup-shaped billet of the second metal. The melting of the billet of said first metal may be just sufficient to wet the interfaces thereof with the cup-shaped second metal or the whole of the first metal may be melted but, in any event, the first and second metals become united at their interfaces to form a unitary composite billet after cooling.

The extrusion of the composite billet can occur with a single blow to form an elongate rod-shaped extrusion having a core of the first metal enclosed substantially entirely within a sheath of the second metal, the side-wall of which is generally thicker in the regions above the end of the copper core than in the region adjacent to this core to provide a suitable volume of the nickel alloy at one end for forming a shoulder thereon. The composite extrusion may be cropped off at one end and the shoulder formed at that end in order to provide mounting means for mounting in the ceramic insulator of a spark plug.

The first metal could be copper and the second metal could be a nickel alloy.

The composite electrode may conveniently be welded to a wire connector by electric butt welding in a known manner, or may be friction welded.

These and other embodiments of the invention will become apparent with reference to the accompanying drawings in which,
Figure 1 is a cross-section through the cup-shaped billet and a further billet contained within the cup.
Figure 2 shows a part-sectional view of the cup-shaped billet contained within a black body,
Figure 3 shows a cross-section of the cup-shaped billet with the copper billet melted inside.
Figure 4 is a cross-sectional view of the composite billet contained within an extrusion die.
Figure 5 is a sectional view of the extruded composite billet and,
Figure 6 is a sectional view of the composite billet having a shoulder portion, and
Figure 7 is a view of the composite electrode of Figure 6 welded to a wire element.

Referring to the drawings, in Figure 1 a cup shaped billet 10 of a heat resistant nickel alloy is of substantially cylindrical shape and has a cylindrical cavity 11 in which has been inserted a copper billet 12, the copper billet having been cropped-off from a length of copper wire (not shown). The cup-shaped billet 10 has a frusto-conical portion 13 at one end thereof comprised solely of nickel alloy.

In Figure 2 is shown a part-sectional view of a rectangular black body 14 of carbon, having a plurality of apertures 15 of cross-sectional shape corresponding substantially to the cross-sectional shape of billet 10. The copper billet 12 is shown contained within a cup-shaped billet 10.

In Figure 3, the copper billet 12 has been melted within the cylindrical part 11 of cup-shaped billet 10 by conduction of heat from a radiant furnace (not shown). The meniscus 16 is of concave section, the peripheral edge of which is joined to the inner surface of billet 10.

Referring to Figure 4, the cup-shaped billet 10 is shown contained within an extrusion die 17 having a cylindrical section 18 of internal diameter corresponding substantially to the external diameter of the billet 10. A converging portion 19 corresponds substantially to the frusto-conical portion of billet 10. An extrusion punch 20 having a frusto-conical end 21 is capable of axial movement downwardly in order to extrude the billet 10 containing the melted copper billet 12 through an extrusion nozzle 22 provided with a clearance 23 of cylindrical shape.

In Figure 5 is shown the extruded billet having an inner core 12 of copper and an outer sheath 10 of nickel alloy substantially entirely enclosing the inner core 12. A flanged head 24 comprised solely of the nickel alloy is formed at one end of the extruded billet 10 which meets at junction 25 to substantially enclose the core 12. The other end of the extruded billet 10 is comprised solely of the nickel alloy, the nickel alloy of this end corresponding generally to the nickel alloy contained within the frusto-conical portion 19 of the billet 10 prior to extrusion.

In Figure 6 the flanged portion 24 of the extrusion has been cropped-off and a shoulder 26 has been formed at one end in order to facilitate mounting within the ceramic insulator of a spark plug. The copper core 12 is still contained substantially entirely within the nickel alloy of billet 10. In Figure 7 a wire element 27 has been connected at 28 to the extrusion adjacent shoulder portion 26, which is comprised entirely of nickel alloy, by electric butt welding in a known way.

In a method of making a centre electrode for a spark plug according to the invention, the cup-shaped biiiet 10 containing the copper billet 12 is placed within a correspondingly shaped recess in the black body 14, which is of carbon, and heated in a radiant furnace having a reducing atmosphere to a temperature at or above the melting point of the copper billet so as to cause melting of the copper billet 12 within the cup-shaped billet 10 to form a composite billet as shown in Figure 3. The composite billet 10, 12 is then placed in the extrusion press as shown in Figure 4 and extruded, by pressure exerted on the billet via punch 20, through nozzle 22 to the shape of a composite electrode as shown in Figure 5. It will be noted that this composite electrode consists of a cigar-shaped inner core 12 of copper and an outer sheath 10 of nickel alloy which substantially entirely encloses the inner core 12 by virtue of part of the metal of cup-shaped billet 10 meeting at 25 subsequent to extrusion. The flanged portion 24 is cropped-off by a cropping machine and a shoulder portion 26 is then formed on this cropped-off end of the billet 10, the shoulder 26 being comprised solely of the nickel alloy.

Since the copper core 12 is substantially entirely enclosed within the nickel alloy sheath 10 a wire element 27 can then be butt welded to the electrode in any known manner, for example by electric butt welding or friction welding to form a welded junction at 28.

It will be apparent from the above that close control of the amount of the first metal contained within the cup-shaped billet of the second metal can be achieved since none of the first metal is extruded out of the sheath of second metal. Thus, a centre electrode is provided according to the invention having closely controlled thermal characteristics which can be simply manufactured and yet is suitable for connection with a wire element as described above.

It will be further apparent that electrodes of different lengths and with different amounts of copper core can be produced by appropriate variations in the volume of copper placed in the cup; and the ratio of cross-section of the copper and nickel alloy composite is determined by the ratio of cylindrical bore to outside diameter of the nickel alloy cup-shaped billet.

## Claims

1. A method of marking a centre electrode for a spark plug of the type having a core (12) of a first metal within a sheath (10) of a second metal, the first metal having a thermal conductivity higher than that of the second metal and a melting point lower than that of the second metal, the second metal being resistive to the corrosive environment in which the electrode works comprising inserting a billet (12) of the first metal within a cup-shaped billet (10) of the second metal and extruding the composite billet to form an elongate rod-shaped extrusion a tip portion of which consists solely of the second metal and an intermediate portion of which consists of said first metal enclosed in said second metal characterised in that:
(a) the two billets (10, 12) are heated together to a temperature at or above the melting point of the first metal but below the melting point of the second metal;
(b) the amount of said first metal (12) in said composite billet is such that when molten it occupies less than the whole of the depth of the cup in said billet (10) of said second metal;
(c) the two metals are cooled to a temperature below the melting point of the first metal to form a composite billet in which the first and second metals are united at their interface; and
(d) when the composite billet is extruded the base portion (24, 25) of the resulting rod-shaped extrusion consists essentially of said second metal whereby the product of said extrusion is a core of the first metal enclosed substantially entirely within a sheath of the second metal.

2. A method according to Claim 1 further characterised in that the heating step comprises heating the two billets (10 and 12) in a reducing atmosphere within a radiant furnace, the cup-shaped billet (10) of the second metal being held in a suitably shaped black body (14) so that conduction of heat from the radiant furnace occurs through the black body in order to melt the billet (12) of the first metal contained within the cup-shaped billet (10) of the second metal.

3. A method according to claim 2 further characterised in that the melting of the billet (12) of the first metal is just sufficient to wet its interfaces with the cup-shaped billet (10) of the second metal.

4. A method according to any one of the preceding claims further characterised in that the extrusion step comprises extruding the composite billet of the first and second metals with a single blow to form the said elongate rod-shaped extrusion having a core of the first metal enclosed substantially entirely within a sheath of the second metal.

5. A method according to any one of the preceding claims further characterised in that the rod-shaped extrusion is cropped off at one end and a shoulder (26) is formed at that end in order to provide mounting means for mounting in the body of a spark plug.

6. A method according to any one of the preceding claims further characterised in that the first metal is copper and that the second metal is a nickel alloy.

## Revendications

1. Procédé pour fabriquer une électrode centrale pour une bougie d'allumage du type comportant un noyau 12 d'un premier métal dans une gaine 10 d'un second métal, le premier métal présentant une conductibilité thermique supérieure à celle du second métal et un point de fusion inférieur à celui du second métal, le second métal résistant au milieu corrosif dans lequel l'électrode travaille, suivant lequel on introduit une billette (12) du premier métal dans une billette en forme de cuvette (10) du second métal et on extrude la billette composite pour former une longue pièce extrudée en forme de broche dont une extrémité est constituée uniquement du second métal et dont une partie intermédiaire est constituée du premier métal enfermé dans le second métal, caractérisé en ce que:
(a) on chauffe les deux billettes (10, 12) ensemble jusqu'à une température égale ou supérieure au point de fusion du premier métal, mais inférieure au point de fusion du second métal;
(b) la quantité du premier métal (12) dans la billette composite est telle que lorsque ce métal est fondu, il occupe moins de la totalité de la profondeur de la cuvette dans la billette (10) du second métal;
(c) on refroidit les deux métaux à une température inférieure au point de fusion du premier métal pour former une billette composite dans laquelle le premier et le second métal sont unis au niveau de leurs interfaces, et
(d) lorsque la billette composite est extrudée, la partie de base (24, 25) de la pièce extrudée en forme de broche résultante est formée essentiellement du second métal, le produit de l'extrusion étant un noyau du premier métal enfermé en substance complètement dans une gaine du second métal.

2. Procédé suivant la revendication 1, caractérisé, en outre, en ce que le stade de chauffage comprend le chauffage des deux billettes (10 et 12) dans une atmosphère réductrice dans un four à rayonnement, la billette en forme de cuvette (10) du second métal étant maintenue dans un corps noir (14) convenablement façonné de sorte que la conduction de la chaleur à partir du four à rayonnement s'effectue à travers le corps noir pour faire fondre la billette (12) du premier métal contenu dans la billette en forme de cuvette (10) du second métal.

3. Procédé suivant la revendication 2, caractérisé, en outre, en ce que la fusion de la billette (12) du premier métal est juste suffisante pour mouiller ses interfaces avec la billette en forme de cuvette (10) du second métal.

4. Procédé suivant l'une quelconque des revendications précédentes, caractérisé, en outre, en ce que le stade d'extrusion comprend l'extrusion de la billette composite du premier et du second métal d'un seul coup pour former la longue pièce extrudée en forme de broche comportant un noyau du premier métal enfermé en substance entièrement dans une gaine du second métal.

5. Procédé suivant l'une quelconque des revendications précédentes, caractérisé, en outre, en ce qu'on sectionne la pièce extrudée en forme de broche à une extrémité et on forme un épaulement (26) à cette extrémité pour fournir des moyens de montage destinés au montage dans le corps d'une bougie d'allumage.

6. Procédé suivant l'une quelconque des revendications précédentes, caractérisé, en outre, en ce que le premier métal est du cuivre et le second métal est un alliage de nickel.

## Patentansprüche

1. Verfahren zur Herstellung einer zentrischen Elektrode für eine Zündkerze des Typs mit einem Kern (12) aus einem ersten Metall innerhalb einer Ummantelung (10) aus einem zweiten Metall, wobei das erste Metall eine thermische Leitfähigkeit aufweist, die höher ist als die des zweiten Metalls und einen Schmelzpunkt, der tiefer ist als der des zweiten Metalls und wobei das zweite Metall widerstandsfähig gegen die korrosive Umgebung ist, in der die Elektrode arbeitet, wobei ein Stück (12) des ersten Metalls in ein topfförmiges Stück (10) des zweiten Metalls eingesetzt und das vereinigte Gebilde zur Formung eines länglichen, stangenförmigen Extrusionsstückes extrudiert wird, wobei ein Spitzenbereich ausschließlich aus dem zweiten Metall besteht und ein Zwischenbereich aus von dem zweiten Metall umhülltem ersten Metall, dadurch gekennzeichnet, daß
(a) die zwei Stücke (10, 12) bei einer Temperatur entsprechend oder oberhalb des Schmelzpunktes des ersten Metalls, jedoch unterhalb des Schmelzpunktes des zweiten Metalls miteinander erhitzt werden;
(b) die Menge des ersten Metalls (12) in dem zusammengesetzten Gebilde derart ist, daß, wenn dieses geschmolzen ist, es weniger als die ganze Tiefe der topfförmigen Höhlung des Stücks (10) aus dem zweiten Metall einnimmt;
(c) die beiden Metalle auf eine Temperatur unterhalb des Schmelzpunktes des ersten Metall les zur Formung eines zusammengesetzten Gebildes heruntergekühlt werden, bei der das erste und das zweite Metall an gegenüberliegenden Flächen miteinander verbunden werden; und
(d) sobald das zusammengesetzte Gebilde extrudiert ist, der Basisbereich (24, 25) des erhaltenen stangenförmigen Extrusionsstückes im wesentlichen aus dem zweiten Metall besteht, wobei als Produkt einer solchen Extrusion ein Kern aus dem ersten Metall erzielt wird, der im wesentlichen vollständig mit einer Umhüllung aus dem zweiten Metall umgeben ist.

2. Verfahren nach Anspruch 1, dadurch gekennzeichnet, daß der Heizschritt ein Aufheizen der zwei Einsatzstücke (10 und 12) in einer reduzierten Atmosphäre in einem Strahlungsofen aufweist, wobei das topfförmige Stück (10) aus dem zweiten Metall in einem geeignet geformten schwarzen Körper (14) gehalten ist, so daß die Wärmeleitung von dem Strahlungsofen über den schwarzen Körper erfolgt, um das Stück (12) aus dem ersten Metall, daß sich in dem topfförmigen Stück (10) aus dem zweiten Metall befindet, zu schmelzen.

3. Verfahren nach Anspruch 2, dadurch gekennzeichnet, daß das Schmelzen des Stückes (12) aus dem ersten Metall gerade ausreichend ist, um die gegenüberliegenden Flächen des topfförmigen Stückes (10) aus dem zweiten Metall zu benetzen.

4. Verfahren nach einem der vorhergehenden Ansprüche, dadurch gekennzeichnet, daß der Extrusionsschritt ein Extrudieren des zusammengesetzten Gebildes aus dem ersten und zweiten Metall mit einer einzigen Umformung zur Formung des länglichen, stangenförmigen Extrusionsstückes einschließt, wobei ein Kern des ersten Metalles im wesentlichen vollständig in einer Ummantelung des zweiten Metalls eingeschlossen ist.

5. Verfahren nach einem der vorhergehenden Ansprüche, dadurch gekennzeichnet, daß das stangenförmige Extrusionsstück an einem Ende gekröpft ausgebildet und eine Schulter (26) zur Bildung von Befestigungsmitteln zur Montage im Körper einer Zündkerze geformt wird.

6. Verfahren nach einem der vorhergehenden Ansprüche, dadurch gekennzeichnet, daß als erstes Metall Kupfer und als zweites Metall eine Nickellegierung verwendet wird.
